

# UNITED STATES PATENT OFFICE.

JOSHUA H. ROBERTSON, OF SAN FRANCISCO, CALIFORNIA, ASSIGNOR TO  
CHARLES W. RANDALL, OF SAME PLACE.

## EXPLOSIVE COMPOUND.

SPECIFICATION forming part of Letters Patent No. 307,989, dated November 11, 1884.

Application filed December 1, 1882. Renewed October 22, 1884. (No specimens.)

*To all whom it may concern:*

Be it known that I, JOSHUA H. ROBERTSON, of the city and county of San Francisco, State of California, have invented a new, useful, and Improved Explosive Compound; and I hereby declare the following to be a full specification of the same; sufficient to enable a person skilled in the art to which my invention appertains to make, compound, and use the same.

My invention consists in combining anhydrous sodium sulphate—commonly known as “sulphate of soda”—with nitro-glycerine, thus forming a new and improved explosive compound; and among the advantages possessed by my compound are diminished cost of production, increased tenacity of union between the ingredients, and a material diminution of noxious fumes. A proportion of nitro-glycerine which, in a compound consisting of infusorial or silicious earth and nitro-glycerine, cannot be exploded, can in my compound be readily and certainly detonated, and, being non-deliquescent, it is not readily affected by moisture.

To produce my compound I place sixty-five (65) pounds of finely-pulverized anhydrous sulphate of soda in a wooden tank or other suitable receptacle, and gradually add thereto thirty-five (35) pounds of nitro-glycerine. I stir the mixture by a wooden rake or other suitable utensil until the nitro-glycerine and sulphate of soda are thoroughly incorporated together, when the compound is ready to be placed into cartridges for use.

I do not desire to limit myself to the proportions of the ingredients herein stated, but give the foregoing as an example merely, the relative proportions being susceptible of considerable change, in accordance with the desired strength or grade of the explosive. The strength of the explosive may be increased or diminished by increasing or diminishing the proportion of nitro-glycerine, the illustration given being taken as a standard, care being taken not to add sufficient nitro-glycerine to reduce the compound to a soft or pasty consistency. When properly prepared, the explosive is of a granular or pulverulent character.

The manner of firing my explosive is the same as that in common use—by means of a detonator, either with or without a priming-charge.

I obtain my anhydrous sulphate of soda at nominal cost by utilizing the waste product known as “niter cake,” resulting from the manufacture of nitric acid, and have found the following process convenient and effective. I place the required quantity of niter cake in a furnace and subject it to a degree of heat sufficient to expel any remaining free acid, which condition can be determined by the usual tests. The product is then dissolved in hot water and allowed to crystallize. The crystals thus obtained are subjected to a degree of heat sufficient to expel the water of crystallization, (about 95° Fahrenheit,) and then ground to an impalpable powder. In this condition the product is ready for use.

I am aware that this process is old, and therefore do not claim it. From whatever source the anhydrous sulphate of soda is obtained, it is essential that any free acid it may contain shall be expelled or neutralized before combining it with the nitro-glycerine.

I am aware that various infusorial, silicious, and volcanic earths have been mixed with nitro-glycerine; also of the United States patent of Shaffner, No. 93,752, in which anhydrous sulphate of lime has been mixed with nitro-glycerine and allowed to set to form a solid mass; also of the United States patent to Fowler, granted February 12, 1878, in which non-hydrated sodium sulphate is described as mixed with other ingredients and with nitro-glycerine.

In an application filed by me in the United States Patent Office February 13, 1884, No. 120,631, and allowed October 18, 1884, I have claimed, broadly, a mixture of granular anhydrous salt and nitro-glycerine, and I claim in this application only the specific elements and in substantially the proportions specified.

Having described my invention, what I claim, and desire to secure by Letters Patent, is—

A new and improved explosive compound, consisting of anhydrous sulphate of soda and nitro-glycerine.

In testimony that I claim the foregoing I have hereunto set my hand and seal this 20th day of November, 1882.

JOSHUA H. ROBERTSON. [L. S.]

Witnesses:

C. W. M. SMITH,  
WM. L. HIGGINS.